# EUROPEAN PATENT SPECIFICATION

(11) **EP 0 545 957 B1**
(45) Date of publication and mention of the grant of the patent: **07.08.1996**
(21) Application number: 91914312.3
(22) Date of filing: 26.08.1991
(51) Int. Cl.: C22C 1/08

(54) **LIGHTWEIGHT METAL WITH ISOLATED PORES AND ITS PRODUCTION**
LEICHTGEWICHTMETALL MIT ISOLIERTEN POREN SOWIE SEINE HERSTELLUNG
METAL LEGER A PORES SEPARES ET PROCEDE DE PRODUCTION

(30) Priority: 27.08.1990 US 573716; 11.07.1991 CA 2046814
(43) Date of publication of application: 16.06.1993
(73) Proprietor: ALCAN INTERNATIONAL LIMITED, Montreal Quebec H3A 3G2 (CA)
(72) Inventor: SANG, Harry 39 Faircrest Blvd., Kingston, Ontario K7L 4V1 (CA); JIN, Iljoon, Kingston, Ontario K7M 5B1 (CA); THOMAS, Martin, Kingston, Ontario K7L 4M6 (CA); KENNY, Lorne, Douglas, Inverary, Ontario K0H 1X0 (CA)
(74) Representative: Gaunt, Robert John
(86) International application number: CA9100300
(87) International publication number: WO9203582

(56) References cited:
- EP-A- 0 151 434
- EP-A- 0 210 803
- WO-A-91/03578
- FR-A- 2 282 479

## Description

This invention relates to a lightweight gas-metal composite with isolated particle-stabilized pores, particularly a lightweight aluminum composite, and its production.

Lightweight foamed metals have high strength-to-weight ratios and are extremely useful as load-bearing materials and as thermal insulators. Metallic foams are characterized by high impact energy absorption capacity, low thermal conductivity, good electrical conductivity and high absorptive acoustic properties.

### Background Art

Foamed metals have been described previously, e.g. in U.S. Patent Nos. 2,895,819, 3,300,296 and 3,297,431. In general such foams are produced by adding a gas-evolving compound to a molten metal. The gas evolves to expand and foam the molten metal. After foaming, the resulting body is cooled to solidify the foamed mass thereby forming a foamed metal solid. The gas-forming compound can be metal hydride, such as titanium hydride, zirconium hydride, lithium hydride, etc. as described in U.S. Patent No. 2,983,597.

A recent development in the production of lightweight foamed metal is described in Jin, U.S. Patent No. 4,973,358, issued November 27, 1990. In that patent, a composite of a metal matrix and finely divided solid stabilizer particles was heated above the liquidus temperature of the metal matrix and gas bubbles were discharged into the molten metal composite below the surface to thereby form a foamed melt on the surface of the molten metal composite. When this foam was cooled, it formed a solid foamed metal having a plurality of closed cells. The cells of this foam were large and had a polygonal structure with quite thin walls between the cells. Such foams in the liquid state are not amenable to shape casting and forming, since the applied forces tend to breakup the fragile cell structure. For example, it is difficult to conformably fill an open mold with this material. Even gentle urgings with a spatula or a similar tool tends to destroy the foam.

It is the object of the present invention to produce a lightweight gas-metal composite which is capable of being subjected to forming procedures without destroying its structural integrity. This object is achieved by the process defined in claim 1. Preferred embodiments of the claimed process are given in the dependent claims.

### Disclosure of the Invention

According to the present invention, a composite of a metal matrix and finely divided solid stabilizer particles is heated above the liquidus temperature of the metal matrix. The molten metal composite is then vigorously mixed such that a vortex is formed. Gas on the surface of the molten metal composite is by way of the action of the vortex drawn into the molten composite. The gas is drawn in as mixing continues such that the hot molten metal composite eventually forms into an expanded material having a pasty or viscous consistency. The gas is distributed throughout this expanded, viscous material in the form of small isolated pores.

This expanded, viscous metal composite material when still above the liquidus temperature of the metal behaves in a very different manner than does the stabilized liquid foam described in U.S. Patent No. 4,973,358. Thus, the hot expanded, viscous material of this invention does not breakup upon the application of an external force. This is so even after the composite has been allowed to stand in the molten condition for an extended period of time (e.g. up to 72 hrs). It is believed that in the interior of the material, the forces are mainly hydrostatic in nature such that only negligible shearing forces occur. However, on the surface the shearing forces are quite strong and the porous structure is destroyed. The result, is a product having a porous interior structure and a smooth exterior skin.

Any of the usual techniques normally applied to either liquids or solids exclusively can be used to shape the small pore three-phase mixtures of this invention. For instance, die-casting may be used, which is normally utilized only with liquids. It is also possible to use thixotropic shaping techniques (M.C. Flemings, Rheocasting, Pages 4241 to 4243 Encyclopedia of Material Sciences and Engineering. Edited by M.B. Bever. Published by Pergamon Press, 1986), such as thixo-extrusion or thixo-forging.

Also, surprisingly the expanded metal product of this invention can be allowed to solidify and can be remelted for forming into a shaped product without breakdown of the expanded structure.

The product of the invention as defined in claim 14 is a stabilized, lightweight metal body comprising a metal matrix having finely divided solid stabilizer particles dispersed therethrough. Also dispersed through the body are a plurality of closed and isolated generally spherical pores having diameters in the range of 50-100 µm, with the stabilizer particles contained in the matrix being concentrated adjacent the interfaces between the matrix metal and the closed pores. The pores are relatively uniformly spaced through the matrix with substantial amounts of matrix material between the pores. In a typical structure, there are widely spaced pores of large diameter with pores of small diameter in the matrix material between the large pores.

The spacing between pores is an average at least 50 µm and typically 100 µm or more. It is an important feature of the present invention that there be a substantial mass of metal composite between the pores. Thus, the product preferably has a relative density (P*/Pₛ) of about 0.3 to ≤ 1, where P* is the density of the porous material and Pₛ is the density of the solid composite.

A wide variety of refractory materials may be used as the finely divided solid stabilizer particles. The main requirements of such particles are that they be capable of being incorporated in and distributed throughout the metal matrix and being capable of at least substantially maintaining their integrity as incorporated rather than losing their form or identity by dissolution in or by extensive chemical combination with the metal matrix.

Examples of suitable solid stabilizer materials include alumina, titanium diboride, zirconia, silicon carbide, silicon nitride, etc. The volume fraction of particles in the foam is typically less than 25% and is preferably in the range of about 5 to 15%. The particle sizes can range quite widely, e.g. from about 0.1 to 50 µm, but generally particle sizes will be in the range of about 0.5 to 25 µm with a particle size range of about 1 to 20 µm being preferred.

The metal matrix may consist of a wide variety of metals capable of being mixed in the molten state by vortex mixing. Examples of these include aluminum, magnesium, steel, zinc, lead, nickel, copper and alloys thereof. Of particular interest are standard wrought, cast or other aluminum alloys, for example alloys available under Aluminum Association (AA) designations 6061, 2024, 7075, 7079 and A 356.

The gas forming the pores may typically be selected from the group consisting of air, carbon dioxide, oxygen, inert gases, etc. Because of its ready availability, air is usually preferred.

The mixing may be done by any means capable of producing a vortex. For instance a mechanical impeller or an electromagnetic mixing system may be used.

In forming the product of the present invention, it has been found that the stabilizer particles adhere to the gas-liquid interface of the pores. This occurs because the total energy of this state is lower than the surface energy of the separate liquid-vapour and liquid-solid state. The presence of the particles around the periphery of the pores tends to stabilize the expanded lightweight material.

The products of this invention are capable of wide industrial application where lightweight metal castings shaped to close dimensional tolerances are required, e.g. parts for the automotive industry.

### Brief Description of the Drawings

Methods and apparatus for performing the present invention will now be more particularly described by way of example with reference to the accompanying drawings in which:
Figure 1 illustrates schematically an apparatus for carrying out the vortex mixing;
Figure 2 shows at 10x magnification a cross-section through a cast lightweight aluminum composite of the invention;
Figure 3 is a photomicrograph of the material of Figure 2 at 100x magnification;
Figure 4 shows at 4x magnification a cross-section through a further cast lightweight aluminum composite according to the invention; and
Figure 5 shows at 25x magnification a cross-section throught part of the product of Figure 4.

### Best Modes For Carrying Out the Invention

In the system shown in Figure 1, a crucible 35 contains a rotatable shaft 36 with an impeller 37. In this particular embodiment, the crucible has a diameter of 32 cm and the blades of the impeller are rectangular, measuring about 76 mm x 127 mm.

In operation, a molten metal composite is filled to the level 38. The impeller is then rotated at high speed to form a vortex 39. A blanket of gas is provided on the surface of the melt vortex, and the gas is drawn into the melt to eventually form an expanded porous material. The expansion is continued until the crucible is substantially filled. At that point, the mixing is stopped and the material is removed from the crucible for forming into desired shapes.

The following non-limiting examples illustrate certain preferred embodiments of the invention.

### Example 1

Using the crucible of Figure 1, A 356 aluminum alloy was melted and 15% by volume of silicon carbide powder was added thereto. The crucible was then evacuated and an atmosphere of argon was provided on the surface of the melt.

With the molten metal composite at a temperature of 650-700°C, the impeller was rotated at 900 rpm. After 10 minutes of mixing, the composite melt started to expand. When the expansion reached the top of the crucible, the impeller was stopped and samples of the expanded, viscous molten material were collected and cast in a sample mould. The cast was sectioned and examined microscopically and the results are shown in the photomicrographs of Figures 2 and 3.

This expanded material was found to have pores which were very small, spherical-shaped and quite evenly distributed. The bulk density of the expanded metal composite material was in the range of 1-1.5 g/cc, with an average pore size of about 250 microns and an average spacing between pores of about 100 microns.

### Example 2

Using the apparatus of Figure 1, a composite of 6061 aluminum alloy reinforced with 15 % by volume of alumina powder was melted. With the molten metal composite at a temperature of 710°C, the impeller was rotated at 800 rpm. After 15 minutes of mixing, the composite melt started to expand and form a viscous molten material. This expanded, viscous molten material was cast in a sample mold. The solidified cast was sectioned and examined microscopically and was found to have an appearance similar to that of the photomicrographs of Figures 2 and 3.

### Example 3

Again using the apparatus of Figure 1, a composite of an aluminum alloy containing 8.5 % by weight of silicon and 10 volume percent silicon carbide powder was melted.

With the molten metal composite at a temperature of 680°C, the impeller was rotated at 1,000 rpm. After about 15 minutes of mixing, the composite melt started to expand. When the material had completed its expansion, the expanded, viscous molten material was cast in a ceramic mold having dimensions of 20 cm x 20 cm x 2.5 cm. A solidified lightweight plate was formed in about 10 minutes and this was sectioned and examined microscopically. A 4x magnification is shown in Figure 4 and it can be seen that evenly distributed spherical shaped pores are present which were not destroyed during the casting operation and which did not coalesce during the slow cooling. From Figure 5, which is a 25x magnification, it can be seen that a molten metal layer is formed at the bottom as a result of drainage, having a thickness of only about 1 mm.

## Claims

1. A process for producing a lightweight gas-metal composite containing isolated particle-stabilized pores, comprising the steps of:
heating a composite of a metal matrix and finely divided solid stabilizer particles above the liquidus temperature of the metal matrix to form a molten metal composite;
mixing the molten metal composite whereby a vortex is formed and continuing the mixing while drawing a gas into the molten composite by way of the vortex until an expanded, viscous molten composite material is formed; and
cooling the expanded material below the solidus temperature of the melt to form a lightweight solid metal product having distributed therethrough a plurality of small isolated, particle-stabilized pores.

2. A process according to claim 1, wherein the stabilizer particles are present in the metal matrix composite in an amount of less than 25% by volume.

3. A process according to claim 2, wherein the stabilizer particles have sizes in the range of about 0.1 to 50 µm.

4. A process according to claim 3, wherein the stabilizer particles have sizes in the range of about 0.5 to 25 µm and are present in the composite in an amount of 5 to 15% by volume.

5. A process according to claim 3, wherein the stabilizer particles are ceramic or intermetallic particles.

6. A process according to claim 3, wherein the stabilizer particles are metal oxides, carbides, nitrides or borides.

7. A process according to claim 3, wherein the stabilizer particles are selected from the group consisting of alumina, titanium diboride, zirconia, silicon carbide and silicon nitride.

8. A process according to claim 3, wherein the mixing is continued until the expanded molten metal composite has a pasty or viscous consistency.

9. A process according to claim 1, wherein the expanded, viscous molten composite material is formed into a shaped, lightweight metal product.

10. A process according to claim 1, wherein the solid metal product is remelted and formed into a shaped, lightweight metal product.

11. A process according to claim 9 or 10, wherein the forming comprises die-casting or thixotropic shaping.

12. A process according to claim 11 wherein the thixotropic shaping is thixo-extrusion or thixo-forging.

13. A process according to claim 1, wherein the metal matrix is aluminum or an alloy thereof.

14. A stabilized, lightweight metal body, comprising:
a metal matrix having finely divided solid stabilizer particles dispersed therethrough; and
said body also having dispersed therethrough a plurality of closed and isolated generally spherical pores having sizes in the range of 10-500 µm, with the stabilizer particles contained in the matrix being concentrated adjacent the interfaces between the matrix metal and the closed pores.

15. A metal body according to claim 14, wherein the pores are spaced from each other by an average distance of about 50 to 100 µm.

16. A metal body according to claim 15, wherein the metal body is a shaped body having smooth outer faces and a core with said spaced pores.

17. A metal body according to claim 15, wherein the stabilizer particles are present in the metal matrix composite in an amount of less than 25% by volume.

18. A metal body according to claim 17, wherein the stabilizer particles have sizes in the range of about 0.1 to 50 µm.

19. A metal body according to claim 18, wherein the stabilizer particles are ceramic or intermetallic particles.

20. A metal body according to claim 19, wherein the metal matrix is aluminium or an alloy thereof.

21. A metal body according to claim 20, wherein the stabilizer particles are metal oxides, carbides, nitrides or borides.

22. A metal body according to claim 14, having a relative density of from about 0.3 to about 1.

## Patentansprüche

1. Verfahren zur Herstellung eines leichtgewichtigen Gas-Metall-Verbundwerkstoffs, der isolierte teilchenstabilisierte Poren enthält, umfassend die Schritte:
Erhitzen eines Verbundwerkstoffs aus einer Metallmatrix und feinverteilten festen Stabilisatorteilchen über die Schmelztemperatur der Metallmatrix zur Bildung eines geschmolzenen Metall-Verbundwerkstoffs;
Mischen des geschmolzenen Metall-Verbundwerkstoffs, wodurch ein Wirbel gebildet wird, und Fortführung des Mischens während ein Gas über den Wirbel in den geschmolzenen Verbundwerkstoff eingesogen wird, bis sich ein ausgedehntes viskoses, geschmolzenes Verbundwerkstoffmaterial gebildet hat; und
Abkühlen des expandierten Materials unter die Erstarrungstemperatur der Schmelze unter Bildung eines leichtgewichtigen festen Metallprodukts mit einer darin verteilten Vielzahl kleiner isolierter teilchenstabilisierter Poren.

2. Verfahren gemäss Anspruch 1, worin die Stabilisatorteilchen in dem Metallmatrix-Verbundwerkstoff in einer Menge von weniger als 25 Vol.% vorhanden sind.

3. Verfahren gemäss Anspruch 2, worin die Stabilisatorteilchen Grössen im Bereich von etwa 0,1 bis 50 µm aufweisen.

4. Verfahren gemäss Anspruch 3, worin die Stabilisatorteilchen Grössen im Bereich von etwa 0,5 bis 25 µm aufweisen und in dem Verbundwerkstoff in einer Menge von 5 bis 15 Vol.% vorhanden sind.

5. Verfahren gemäss Anspruch 3, worin die Stabilisatorteilchen keramische oder intermetallische Teilchen sind.

6. Verfahren gemäss Anspruch 3, worin die Stabilisatorteilchen Metalloxide, Carbide, Nitride oder Boride sind.

7. Verfahren gemäss Anspruch 3, worin die Stabilisatorteilchen ausgewählt sind aus Aluminiumoxid, Titandiborid, Zirkonoxid, Siliciumcarbid und Siliciumnitrid.

8. Verfahren gemäss Anspruch 3, worin das Mischen fortgeführt wird, bis der expandierte geschmolzene Metall-Verbundwerkstoff eine pastöse oder viskose Konsistenz besitzt.

9. Verfahren gemäss Anspruch 1, worin das expandierte viskose, geschmolzene Verbundwerkstoffmaterial zu einem geformten leichtgewichtigen Metallprodukt ausgebildet wird.

10. Verfahren gemäss Anspruch 1, worin das feste Metallprodukt umgeschmolzen und zu einem geformten leichtgewichtigen Metallprodukt ausgestaltet wird.

11. Verfahren gemäss Anspruch 9 oder 10, worin die Formgebung Formgiessen oder thixotrope Formgebung umfasst.

12. Verfahren gemäss Anspruch 11, worin die thixotrope Formgebung Thixoextrusion oder Thixoschmiedung ist.

13. Verfahren gemäss Anspruch 1, worin die Metallmatrix Aluminium oder eine Legierung davon ist.

14. Stabilisierter leichtgewichtiger Metallkörper, umfassend eine Metallmatrix mit darin dispergierten, feinverteilten, festen Stabilisatorteilchen; und besagter Körper weist ebenso darin dispergiert eine Vielzahl an geschlossenen und isolierten, im allgemeinen sphärischen Poren mit Grössen im Bereich von 10 bis 500 µm auf, die in der Matrix enthaltenen Stabilisatorteilchen sind in der Umgebung der Grenzflächen zwischen dem Matrixmetall und den geschlossenen Poren konzentriert.

15. Metallkörper gemäss Anspruch 14, worin die Poren durch eine durchschnittliche Distanz von etwa 50 bis 100 µm voneinander räumlich getrennt sind.

16. Metallkörper gemäss Anspruch 15, worin der Metallkörper ein geformter Körper mit glatten Aussenflächen und einem Kern mit den besagten, räumlich getrennten Poren ist.

17. Metallkörper gemäss Anspruch 15, worin die Stabilisatorteilchen in dem Metallmatrix-Verbundwerkstoff in einer Menge von weniger als 25 Vol.% vorhanden sind.

18. Metallkörper gemäss Anspruch 17, worin die Stabilisatorteilchen Grössen im Bereich von etwa 0,1 bis 50 µm aufweisen.

19. Metallkörper gemäss Anspruch 18, worin die Stabilisatorteilchen keramische oder intermetallische Teilchen sind.

20. Metallkörper gemäss Anspruch 19, worin die Metallmatrix Aluminium oder eine Legierung davon ist.

21. Metallkörper gemäss Anspruch 20, worin die Stabilisatorteilchen Metalloxide, Carbide, Nitride oder Boride sind.

22. Metallkörper gemäss Anspruch 14, der eine relative Dichte von etwa 0,3 bis etwa 1 aufweist.

## Revendications

1. Procédé de production d'un composite gaz-métal léger contenant des pores isolés stabilisés par des particules, comprenant les étapes consistant à:
chauffer un composite constitué d'une matrice métallique et de particules stabilisatrices solides finement divisées à une température supérieure à la température de liquidus de la matrice métallique afin de former un composite métallique fondu;
mélanger le composite métallique fondu, formant ainsi un tourbillon, et continuer à mélanger tout en attirant un gaz dans le composite fondu par l'intermédiaire du tourbillon jusqu'à ce qu'un composite fondu visqueux expansé se forme; et
refroidir le matériau expansé à une température inférieure à la température de solidus de la fusion afin de former un produit métallique solide léger dans lequel est répartie une pluralité de petits pores isolés stabilisés par des particules.

2. Procédé selon la revendication 1, dans lequel les particules stabilisatrices sont présentes dans le composite à matrice métallique avec une teneur inférieure à 25% en volume.

3. Procédé selon la revendication 2, dans lequel les particules stabilisatrices ont une taille comprise entre 0,1 et 50 µm environ.

4. Procédé selon la revendication 3, dans lequel les particules stabilisatrices ont une taille comprise entre 0,5 et 25 µm environ et sont présentes dans le composite avec une teneur de 5 à 15% en volume.

5. Procédé selon la revendication 3, dans lequel les particules stabilisatrices sont des particules céramiques ou intermétalliques.

6. Procédé selon la revendication 3, dans lequel les particules stabilisatrices sont des oxydes, des carbures, des nitrures ou des borures métalliques.

7. Procédé selon la revendication 3, dans lequel les particules stabilisatrices sont choisies parmi le groupe comprenant l'alumine, le diborure de titane, la zircone, le carbure de silicium et le nitrure de silicium.

8. Procédé selon la revendication 3, dans lequel le mélange est poursuivi jusqu'à ce que le composite métallique fondu expansé ait une consistance pâteuse ou visqueuse.

9. Procédé selon la revendication 1, dans lequel le matériau composite visqueux expansé est formé en un produit métallique léger profilé.

10. Procédé selon la revendication 1, dans lequel le produit métallique solide est fondu à nouveau et formé en un produit métallique léger profilé.

11. Procédé selon la revendication 9 ou la revendication 10, dans lequel le formage comprend le moulage sous pression ou le profilage thixotrope.

12. Procédé selon la revendication 11, dans lequel le profilage thixotrope est la thixo-extrusion ou le thixo-forgeage.

13. Procédé selon la revendication 1, dans lequel la matrice métallique est l'aluminium ou un alliage d'aluminium.

14. Corps métallique léger stabilisé comprenant:
une matrice métallique dans laquelle sont dispersées des particules stabilisatrices solides finement divisées; et
une pluralité de pores fermés et isolés, généralement sphériques, ayant des tailles de l'ordre de 10 à 500 µm, également dispersés dans ledit corps, les particules stabilisatrices contenues dans la matrice étant concentrées au voisinage des interfaces entre la matrice métallique et les pores fermés.

15. Corps métallique selon la revendication 14, dans lequel les pores sont espacés les uns des autres d'une distance moyenne de 50 à 100 µm environ.

16. Corps métallique selon la revendication 15, dans lequel le corps métallique est un corps profilé ayant des faces externes lisses et un noyau avec lesdits pores espacés.

17. Corps métallique selon la revendication 15, dans lequel les particules stabilisatrices sont présentes dans le composite à matrice métallique avec une teneur inférieure à 25% en volume.

18. Corps métallique selon la revendication 17, dans lequel les particules stabilisatrices ont des tailles comprises entre 0,1 et 50 µm environ.

19. Corps métallique selon la revendication 18, dans lequel les particules stabilisatrices sont des particules céramiques ou intermétalliques.

20. corps métallique selon la revendication 19, dans lequel la matrice métallique est l'aluminium ou un alliage d'aluminium.

21. Corps métallique selon la revendication 20, dans lequel les particules stabilisatrices sont des oxydes, des carbures, des nitrures ou des borures métalliques.

22. Corps métallique selon la revendication 14, ayant une densité relative comprise entre environ 0,3 et environ 1.
